

## UNITED STATES PATENT OFFICE

BERNHARD QUENDT, OF ESSEN, GERMANY

## PRELIMINARY TANNING PROCESS

No Drawing. Application filed January 25, 1929, Serial No. 335,141, and in Germany July 19, 1926.

The present invention relates to a process for preliminary treating hides for promoting the tanning thereof and preparations therefor, and for which I applied for patent in Germany July 19, 1926.

A preliminary treatment of hides, for tanning, with alum and sodium chloride and in some cases by the addition of chrome alum is already known.

10 The resulting advantage of such combination tanning consists only in an acceleration of the tanning and perhaps in a special grain. Nevertheless the leather cannot be spoken of as purely bark tanned on account 15 of the fact that it exhibits peculiarities which are absent from a bark tanned leather, tendency to stretch for example.

It has now been found that the tanning particularly the vegetable tanning of hides 20 may be accelerated without alteration in the character of the leather if in the preliminary treatment a water soluble condensation product of an aromatic amine be added the salt of an aromatic amine or preferably a water 25 soluble condensation product of a secondary or tertiary aromatic amine be added to the alum and one or more neutral salts, for example to the alum and sodium chloride, or to the alum, Glauber's salt and sodium 30 chloride, or to a quebracho liquid, or other vegetable tanning liquid, or even to clear water.

By such preliminary treatment of the hides according to the present invention the 35 penetration of the tan in the tanning, particularly the vegetable tanning, process is promoted and a better tanning is realized.

An example of the use of a salt of an aromatic amine for the preliminary treatment 40 of the hides under the present invention which serve well is as follows:

## Example 1

430 parts by weight of alum, 200 parts by 45 weight each of Glauber's salt and sodium chloride, 10 parts by weight of aniline hydrochloride, 2 parts by weight of potassium carbonate and 5 parts by weight of potassium ferricyanide are mixed, either in the 50 form of dry powder or in the form of solu-

tion and are then diluted at 5° Baumé. To this solution is then added 5 parts by weight of 55 30% formaldehyde which forms a complex water soluble condensation product with the other ingredients. In this solution the hides receive their preliminary treatment either in a tumbler-drum or in a suspending vat. In the tumbler-drum the treatment lasts about 12 hours; if the hides are suspended they should hang in the liquid 60 for 24 to 48 hours. The skins are then washed for 10 minutes and go into the vegetable tanning liquid which must be at 5° Baumé. The leather after tanning is dried and finished according to usual or approved 65 methods.

In the case of upper leather or leather of that character this, after it has been thoroughly tanned, is again washed and then dried and finished according to usual or approved 70 methods to bring the leather to its final colour, texture, grain or other desired condition.

## Example 2

5 parts by weight of dimethylaniline are 75 condensed with 4 parts by weight of monochloracetic acid and 2 parts by weight formaldehyde (30%). The condensation product is mixed with 400 parts by weight of alum and 200 parts by weight each of Glauber's 80 salt and sodium chloride. This also is employed as a solution of 5° Baumé. The treatment and subsequent tanning is carried out in accordance with Example 1.

## Example 3

The condensation product given in Example 2, which is a viscous liquid, is added to clear water or, otherwise, to a quebracho liquid or other tanning solution having a 90 strength of about 1° to 3° Baumé. The proportion of the condensation product should be in the ratio of 0.5 to 0.3% by weight of the water or Tanning liquor. In this solution the hide is treated as in Example 1 but 95 only for about 3 to 5 hours. The hides are afterwards placed for about 10 hours in a strong vegetable or other tanning solution of about 5° to 8° Baumé. The further treatment then follows according to Example 1. 100

*Example 4*

The condensation product detailed in Example 2 is mixed with vegetable or other tanning solution and put into water in a suspending vat. The solution so made may by way of example be a 0.5 to 0.3% by weight solution, and also by way of example the mixture of the condensation product and the solution may be in the proportions of 1 part by weight of the condensation product to from 1 to 4 parts by weight of the solution.

The hides remain in this solution (as in Example 1) for about one to two days (24-48 hours) after which they are tanned and finally finished as in Example No. 1.

If this Example 4 is carried out in a tumbler-drum the tanner will know the weight of hide which can be treated in a given drum and the conditions governing the water content thereof. He will therefore calculate the weight of the hide and add an amount of the mixture of the condensation product and extract equal in weight to 1 to 3% of the said weight of the hide to be treated in the drum.

The hides will remain in the solution in the drum for from four to five hours.

In some cases the preliminary treatment hereinabove referred to may be carried out prior to any treatment or between the treatment of the hides in the first and second, or second and third, or third and fourth tanning vats, the usual preparatory or beam house processes.

After the preliminary treatment as described and as detailed in Examples 1 to 4, the hides may be subjected to the customary tanning processes using the ordinary strong tanning solutions, which it will be found will more quickly and effectually penetrate the hides preliminarily treated by the process and with the preparations as described in this invention.

The time of the tanning which is accelerated by the present invention will of course vary in accordance with the thickness and hardness of the hide.

As an example of how a condensation or product is prepared, 5 parts by weight of dimethylaniline and 4 parts by weight of monochloracetic acid are so mixed by a stirrer in hot water that they are brought to a thin solution. This solution is then heated to 100° C. for 2 hours while being stirred. The solution is allowed to cool down to 70-80° C. and then 2 parts by weight of formaldehyde is added. The resulting mixture is then stirred for about 5 minutes and put into an autoclave and treated for about 3 hours at a pressure of  $\frac{1}{10}$  of an atmosphere over atmosphere until the final product is well thickened.

What I claim is:

1. Process for promoting the tanning of hides by subjecting the hides, after the usual

preparatory processes, to a preliminary treatment with a solution of a water soluble non-sulphonated condensation product of an aromatic amine.

2. Process for promoting the tanning of hides by subjecting the hides, after the usual preparatory processes, to a preliminary treatment with a mixture of neutral salts, and a water soluble non-sulphonated condensation product of an aromatic amine. 75

3. Process for promoting the tanning of hides by subjecting the hides, after the usual preparatory processes, to a preliminary treatment with a mixture of alum, a neutral salt, and a water soluble non-sulphonated condensation product of an aromatic amine. 80

4. Process for promoting the tanning of hides by subjecting the hides, after the usual preparatory processes, to a preliminary treatment with a mixture of a water soluble non-sulphonated condensation product of an aromatic amine and a weak tanning solution. 85

In testimony whereof, I affix my signature.

BERNHARD QUENDT.

90

95

100

105

110

115

120